

## UNITED STATES PATENT OFFICE

2,241,803.

## MOTTLED ENAMELWARE

Eugene E. Bryant, Bedford, Ohio, assignor to  
 Ferro Enamel Corporation, Cleveland, Ohio, a  
 corporation of Ohio

No Drawing. Application November 7, 1938,  
 Serial No. 239,336

15 Claims. (Cl. 91—73)

This invention, as indicated, relates to mottled enamelware and a method of producing the same.

The term "mottled," as used herein, is descriptive of a porcelain enamel coating possessing an irregular lacy pattern resulting from a surface ornamentation of the base metal over which the enamel is applied. The surface ornamentation most commonly resorted to in producing mottled ware is a controlled "rusting" of the ferrous base over which the protective enamel coating is applied.

It has been found that the controlled "rusting" of the metal base, in order to secure the mottled appearance, may be effected either prior to the application of the enamel or by means of a constituent in the wet enamel slip applied to the ware.

Irrespective of which procedure has been followed, a period up to about 24 hours has been required in order to effect a sufficient amount of rusting of the work that the proper mottled appearance might be produced. It has, therefore, been common practice to incorporate the rusting agent in the enamel slip and to then very slowly dry the green work for a period of about 2 to 24 hours during which time the rusting constituent in the slip performs its function and at the end of which time the green and then dried work may be fired in a muffle to produce the fused enamel coating through which the pattern of the rusted surface of the work shows, in providing the mottled appearance of the latter.

There are two principal objections to this prior art procedure which is now commonly followed, in that enamels of high final gloss have not been adapted for use with such process and the long drying period of the green work has necessitated extra storage space and additional handling.

It is, therefore, a principal object of this invention to provide a method of producing a mottled appearing enamel surface without the necessity of a long drying period to allow the corrosive material to act.

A further object is to provide a method of obtaining a mottled appearing enamel surface of a high gloss.

Other objects of the invention will appear as the description proceeds.

To the accomplishment of the foregoing and related ends, said invention, then consists of the steps hereinafter fully described and particularly pointed out in the claims. The following description sets forth in detail one approved method of carrying out the invention, such disclosed method, however, constituting but one of the ways in

which the principle of the invention may be employed.

In general, my invention comprises the discovery that a fully satisfactory mottled appearance may be imparted in a very short time to the ferrous work surface, prior to the application of the enamel thereon, by the use of suitable reagents under properly controlled conditions so that the enamel, when applied to the work, may be immediately dried and fired and the entire process of producing mottled enamelware reduced to a substantially continuous sequence of steps without the necessity of storing the work in order to develop the mottled appearance.

In general, my invention comprises the steps of treating the ferrous surface of the article to be enamelled with a selected corrosive solution under properly controlled temperature conditions for a predetermined length of time, passivating the surface after such treatment and then applying the enamel.

The process comprising my invention for "mottling" the ware is performed after the ware has been otherwise prepared as by pickling or acid treatment for the reception of the enamel coat. General care should be exercised to clean the ware prior to subjecting the same to the steps comprising my process for mottling, in particular, any excess acid or the like adhering to the work from the conventional pickling step should be rinsed or soaked therefrom.

The controlled rusting process forming a part of my invention may be performed either before or after the customary neutralizing step during which any acid remaining on the work and which might interfere with the successful application of enamel is neutralized by means of an alkali bath.

To the ware thus properly pickled, and, as indicated, either before or after the neutralizing step, I apply a corrosive aqueous solution of a sulphate, preferably by dipping in the solution. The sulphate which is used may be either sodium sulphate, nickel sulphate or copper sulphate. If sodium sulphate is employed, the same may be added to the solution in the form of commercial Glauber's salt, since the impurities in such commercial material are not detrimental. I have found that a rather close control over the concentration of the sulphate in the aqueous solution is necessary. When sodium sulphate is employed, an aqueous solution of 1% to 4% of the same will be found to produce most satisfactory results. When nickel sulphate is employed, an aqueous solution of from 1/2% to 3% will be found

to work best and when copper sulphate is employed concentrations of from 1% to 4% will be found most satisfactory.

Inasmuch as the mottled appearance of the work is due to the generation thereon of an oxide film which film later combines with the enamel to produce the mottled effect, minor amounts of an oxidizing agent added to the solution will be found useful. Oxidizing agents such as potassium sulphide (potassium sulphuret) and sodium sulphide employed in amounts of about 1 to 2 ounces to 100 gallons of solution have been found to aid in the production of a heavy and thus more distinctive mottle. These alkali sulphides may be present in the form of a mixture of the various sulphides. Various other oxidizing agents may be employed such as potassium dichromate and potassium permanganate but the alkali sulphides above indicated will generally be preferred.

I have found that in order to produce a mottled appearance of the desired character and in the desired time, the pH of the corrosive solution should be rather carefully controlled. I have found that the pH of the corrosive aqueous solution employing any of the sulphates above mentioned should range from about 5 to 8 or sometimes 8.5 and generally from 6.5 to 7.5 for best results. Too low a pH value produces a rusting of such intensity that actually no mottle design is produced and when the pH value is too high, no mottle at all is produced. When sodium sulphate is employed, the preferable pH range is from 7 to 7.5. When nickel sulphate or copper sulphate is employed, the preferable pH range is from about 7 to about 8.

Various agents may be employed to regulate the pH of the solution such as sodium bicarbonate, ammonium hydroxide, and ammonium carbonate, of which sodium bicarbonate is preferred, since it sets up a buffer solution with the result that the pH value holds constant for a longer period of time. When it is desired to use an agent such as ammonium carbonate, as when the corrosive solution contains nickel sulphate, a small amount of sodium bicarbonate may also be added as a buffer to aid in holding the pH value constant.

Any electrolyte that has a corrosive action on steel when in a solution adjusted to a pH of from about 5 to 8.5 will produce the desired mottled effect but sulphates are generally preferred since their use seems to cause the least defects in the enamel surface. A mixture of sulphates, such as a mixture of sodium sulphate and nickel sulphate, gives excellent results. The chlorides such as NaCl, KCl, CaCl<sub>2</sub>, the nitrates, etc., whether added as such or produced in the bath by the addition of acids and pH control agents, will be found to be satisfactory insofar as the production of a mottled surface is concerned but are generally less desirable than the sulphates due to their tendency to adversely affect the enamel. Mixtures of chlorides and sulphates may also be employed with generally improved results over those obtained when the chlorides are employed alone.

From the corrosive solution the ware next passes to a steam closet where it is allowed to remain until the desired degree of mottling is obtained. Any moist or non-drying atmosphere greatly accelerates this rusting process which is also furthered by the application of heat. The use of steam provides an effective and inexpensive method of affording the proper conditions

of moisture and temperature, care being taken that a certain amount of air is always mixed and circulated with the steam. The temperature may be maintained at any figure from room temperature up to about 250° F. and preferably at from about 150° F. to 185° F. The higher the temperature the more rapid the rusting but there is some danger of sudden drafts quickly drying the ware at the higher temperatures. Also, to prevent condensation on the ware when it enters the steam closet which would result in the condensate washing from the work the film relied upon to produce the mottled design, the ware should be at a temperature approximately equal to that maintained in the closet and this necessitates heating the corrosive solution from which the ware passes to the steam closet.

When corrosive solutions of the preferred concentrations and preferred pH are applied to the work and the latter subjected to the substantially non-drying atmosphere maintained at the preferred temperature range, a very satisfactory mottle will be produced in from about 5 to 15 minutes. In this way, the step of mottling the work is reduced to the point where it may be performed while the ware passes practically continuously through a general plant for the production of porcelain enamelled articles. No storage is necessary and, therefore, expensive storage facilities need not be provided and the expense of rehandling is eliminated.

If the concentration of the corrosive solution is changed from the preferred ranges above given in order, for example, to produce a slightly different form of mottled appearance, the time required for the corrosive solution to act may be somewhat lengthened. In general, the best results will be produced by solutions which will act to produce the desired effect in a period not substantially in excess of 30 to 45 minutes, and usually such desired result may be obtained in less than 15 minutes.

Following the above treatment, the ware should be rinsed, first, in water and then in a neutralizer solution to remove any material harmful to enameling. The mottled surface may be passivated, usually by a mild alkali wash and then a rinse in clear water. After drying, the ware may then be enamelled by a normal procedure employing a relatively clear enamel which will permit the mottle design to show through. Much clearer enamels and enamels with much higher gloss may be used than those generally applied in the past to make the usual gray or mottled ware so that the finished ware is considerably improved in appearance. A color may be produced which is distinctly different from the ordinary gray.

The enamel which is applied over the mottled surface of the work prepared in accordance with the principles of my invention may be a substantially clear porcelain enamel of the following general formula:

|                   | Percent |
|-------------------|---------|
| Anhydrous borax   | 22      |
| Feldspar          | 28      |
| Quartz            | 28      |
| Soda ash          | 9       |
| Sodium nitrate    | 5       |
| Fluorspar         | 5       |
| Calcium carbonate | 3       |

The enamel, converted into a slip in accordance with conventional practice is applied to

the mottled surface by conventional means such as dipping or spraying and the ware then fired at the usual temperatures as the last step in the complete process.

The above described process may, as indicated, form a part of a substantially continuous process for the production of mottled enamelled ware, and the following is a brief outline of the various steps comprising such continuous process.

The ware, as it is received from the forming machines or presses, is racked in suitable baskets of the type usually employed in handling ware of this character. The baskets of ware, unless previously degreased, are soaked in a cleaner tank to remove grease and dipped in a wash tank to remove the cleaning fluid. Then the baskets of ware are immersed in a pickling solution for the purpose of cleaning the surface thereof in order that the enamel may be properly bonded thereto. The pickling solution usually contains an amount of iron sulphate which, as the basket is removed from the pickling tank, will deposit a slight scum on the surface of the ware. In order to remove this scum, the basket is next dipped in a mild acid rinse which removes all foreign material from the surface of the ware. The baskets of ware are then preferably dipped in a wash tank for the purpose of removing any excess amount of acid adhering to the work. At this point, what is commonly known as a nickel dip treatment, may be used to improve the bonding of the porcelain enamel. This treatment is followed by one or more wash tanks. It is, of course, necessary to passivate the surface of the work before any enamel is applied thereto, such passivating step usually comprising an alkali wash for the purpose of neutralizing the acid surface of the ware. The mottling step comprising one feature of my invention may, as indicated, be performed either before or after this passivating step, but since a certain amount of corrosion of the ware takes place during the mottling step, I prefer to carry on the various steps of the general process in such sequence that the mottling step immediately precedes a final passivating step.

The mottling step of the general process consists in dipping the baskets containing the cleaned ware as received from the above described treatment into the mottling solution and from this tank the baskets are then placed in another tank, usually covered, in the bottom of which is maintained a water bath in order to provide the non-drying atmosphere within which the work is corroded to produce the mottled design. This tank has been referred to hereinbefore as a steam closet.

The baskets of ware removed from the steam closet are next immersed in passivating solutions which may be a clear water rinse and a mild alkaline rinse, and after being removed therefrom, the ware is dried and is ready to be enamelled; the enamelling step comprising either dipping or spraying the ware with a slip of the character above defined after which the ware is immediately dried and may be promptly fired.

As above indicated, the principal advantage derived from the employment of the process of this invention is that the enamel does not require a long drying period and production is correspondingly accelerated. Also, the improved appearance of the finished product enlarges the demand for this type of ware.

It is to be understood, of course, that this process may be employed whenever a mottled

appearing enamelled surface is desired and is not limited to the production of kitchenware and the like.

Other modes of applying the principle of my invention may be employed instead of the one explained, change being made as regards the method herein disclosed, provided the step or steps stated by any of the following claims or the equivalent of such stated step or steps be employed.

I, therefore, particularly point out and distinctly claim as my invention:

1. The method of producing a mottled appearing enamel surface which comprises coating the surface of a ferrous article to be enamelled with a corrosive solution of an electrolyte having a pH ranging from 5 to 8, maintaining said surface in a substantially moisture-saturated atmosphere until a well-defined mottled surface is produced, rinsing and passivating the mottled surface coating the article with a vitreous enamel slip and then firing the enamel.

2. The method of producing a mottled appearing enamel surface which comprises coating the surface of a ferrous article to be enamelled with a corrosive solution of an electrolyte having a pH ranging from 5 to 8, maintaining said surface in a heated substantially moisture-saturated atmosphere for a period on the order of about five to about thirty minutes, rinsing and passivating the mottled surface coating the article with a vitreous enamel slip and then firing the enamel.

3. The method of producing a mottled appearing enamel surface which comprises coating the surface of a ferrous article to be enamelled with a corrosive solution of an electrolyte having a pH ranging from 6.5 to 7.5, maintaining said surface in a substantially moisture-saturated atmosphere at a temperature of from about 150° to 250° F. for a period of from five to fifteen minutes until a well-defined mottled surface is produced, rinsing and passivating the mottled surface coating the article with a vitreous enamel slip and then firing the enamel.

4. The method of producing a mottled appearing enamel surface which comprises coating the surface of a ferrous article to be enamelled with a solution of corroding and oxidizing agents having a pH ranging from 5 to 8, maintaining said surface in a substantially moisture-saturated atmosphere at a temperature of from about 150° to 185° F. until a well-defined mottled surface is produced, rinsing and passivating the mottled surface coating the article with a vitreous enamel slip and then firing the enamel.

5. The method of producing a mottled appearing enamel surface which comprises coating the surface of a ferrous article to be enamelled with a corrosive solution of sulphate having a pH ranging from 5 to 8, maintaining said surface in a substantially moisture-saturated atmosphere at a temperature of from about 150° to 250° F. until a well-defined mottled surface is produced, rinsing and passivating the mottled surface coating the article with a vitreous enamel slip and then firing the enamel.

6. The method of producing a mottled appearing enamel surface which comprises coating the surface of a ferrous article to be enamelled with a corrosive solution of a sulphate and an alkali sulphide having a pH ranging from 5 to 8, maintaining said surface in a substantially moisture-saturated atmosphere at a temperature of from about 150° to 250° F. for a period not longer than

one hour but until a well-defined mottled surface is produced, rinsing and passivating the mottled surface coating the article with a vitreous enamel slip and then firing the enamel.

7. The method of producing a mottled appearing enamel surface which comprises coating the surface of a ferrous article to be enamelled with a corrosive solution of sodium sulphate having a pH ranging from 5 to 8, maintaining said surface in a substantially moisture-saturated atmosphere at a temperature of from about 150° to 250° F. for a period not longer than one hour but until a well-defined mottled surface is produced, rinsing and passivating the mottled surface coating the article with a vitreous enamel slip and then firing the enamel.

8. The method of producing a mottled appearing enamel surface which comprises coating the surface of a ferrous article to be enamelled with a corrosive solution of sodium sulphate having a pH ranging from about 6.5 to 7.5, maintaining said surface in a substantially moisture-saturated atmosphere at a temperature of from about 150° to 185° F. until a well-defined mottled surface is produced, rinsing and passivating the mottled surface coating the article with a vitreous enamel slip and then firing the enamel.

9. The method of producing a mottled appearing enamel surface which comprises coating the surface of a ferrous article to be enamelled with a corrosive solution of sodium sulphate having a pH ranging from 5 to 8, maintaining said surface in a substantially moisture-saturated atmosphere at a temperature of from about 150° to 185° F. for a period of from 5 to 15 minutes, rinsing and passivating the mottled surface coating the article with a vitreous enamel slip and then firing the enamel.

10. The method of producing a mottled appearing enamel surface which comprises coating the surface of a ferrous article to be enamelled with a corrosive solution of sodium sulphate having a pH ranging from 5 to 8 and containing a minor amount of an oxidizing agent, maintaining said surface in a substantially moisture-saturated atmosphere at a temperature of from about 150° to 250° F. for a period not longer than one hour but until a well-defined mottled surface is produced, rinsing and passivating the mottled surface coating the article with a vitreous enamel slip and then firing the enamel.

11. The method of producing a mottled appearing enamel surface which comprises coating the surface of a ferrous article to be enamelled with a corrosive solution of nickel sulphate hav-

ing a pH ranging from 5 to 8, maintaining said surface in a substantially moisture-saturated atmosphere at a temperature of from about 150° to 250° F. until a well-defined mottled surface is produced, rinsing and passivating the mottled surface coating the article with a vitreous enamel slip and then firing the enamel.

12. The method of producing a mottled appearing enamel surface which comprises coating the surface of a ferrous article to be enamelled with a corrosive solution of nickel sulphate having a pH ranging from about 6.5 to 7.5, maintaining said surface in a substantially moisture-saturated atmosphere at a temperature of from about 150° to 185° F. for a period of about 5 to 15 minutes, rinsing and passivating the mottled surface coating the article with a vitreous enamel slip and then firing the enamel.

13. The method of producing a mottled appearing enamel surface which comprises coating the surface of a ferrous article to be enamelled with a corrosive solution of nickel sulphate having a pH ranging from about 6.5 to 7.5, and containing a minor amount of potassium sulphide, maintaining said surface in a substantially moisture-saturated atmosphere at a temperature of from about 150° to 185° F. for a period of from 5 to 15 minutes, rinsing and passivating the mottled surface coating the article with a vitreous enamel slip and then firing the enamel.

14. The method of producing a mottled appearing enamel surface which comprises coating the surface of a ferrous article to be enamelled with a corrosive solution of copper sulphate having a pH ranging from 5 to 8, maintaining said surface in a substantially moisture-saturated atmosphere at a temperature of from about 150° to 250° F. until a well-defined mottled surface is produced, rinsing and passivating the mottled surface coating the article with a vitreous enamel slip and then firing the enamel.

15. The method of producing a mottled appearing enamel surface which comprises coating the surface of a ferrous article to be enamelled with a corrosive solution of copper sulphate having a pH ranging from about 6.5 to 7.5 and containing a minor amount of an oxidizing agent, maintaining said surface in a substantially moisture-saturated atmosphere at a temperature of from about 150° to 185° F. for a period of from 5 to 15 minutes, rinsing and passivating the mottled surface coating the article with a vitreous enamel slip and then firing the enamel.

EUGENE E. BRYANT.